

L. HAMBURGER AND D. LELY, JR.  
ELECTRIC INCANDESCENT LAMP,  
APPLICATION FILED JAN. 11, 1917.

1,317,492.

Patented Sept. 30, 1919.



WITNESS :

*Reine Blaue*  
*Gustav R. Thompson*

INVENTORS :

*Lodewijk Hamburger and*  
*Dirk Lely, Junior*  
By Attorneys,

*Fraser, Turst & Nevers*

# UNITED STATES PATENT OFFICE.

LODEWIJK HAMBURGER AND DIRK LELY, JR., OF EINDHOVEN, NETHERLANDS.

## ELECTRIC INCANDESCENT LAMP.

1,317,492.

Specification of Letters Patent. Patented Sept. 30, 1919.

Application filed January 11, 1917. Serial No. 141,840.

To all whom it may concern:

Be it known that we, LODEWIJK HAMBURGER and DIRK LELY, Jr., subjects of the Queen of the Netherlands, residing at Eindhoven, Kingdom of the Netherlands, have invented new and useful Improvements in or Relating to Electric Incandescent Lamps; and we do hereby declare the following to be a full, clear, and exact description of the same.

In many electric incandescent lamps, for instance, those having a tungsten filament, the temperature to which the filament may be raised under high vacuum, is not limited by the melting point of the metal, but by its vapor pressure, because under such conditions of temperature and vacuum the vaporized metal condenses upon the bulb and obscures it. It has been proposed to prevent this obscuring of the bulb by introducing substances into the lamp which during its burning evolved gases which reacted with the vaporized or atomized particles of the filament, to form compositions which do not obscure the light as much as the condensed filament vapors. In the case of tungsten filament lamps this may be effected, for instance, by halogen or oxygen compounds. The aforesaid substances have been placed in the lamp in locations of greater or less heat in accordance with their volatility or decomposability.

It has been found however that many substances which even at high temperatures do not give off any reacting vapor, such as oxid of sodium  $Na_2O$ , sodium phosphate  $Na_3PO_4$ , the fluorids of the metals of the alkaline earths and silica,  $SiO_2$ , nevertheless may have a beneficent influence upon the duration of the useful life of the lamp. This has proven to be the case and in like degree even when a lamp, containing said substances only upon the inner walls of the bulb, was burnt while being immersed in liquid air. The same action, the retarding of the obscuring of the bulb, was also found when in lieu of a tungsten filament, filaments of other elements, for instance, carbon, molybdenum, platinum, iron, silver, zinc or copper were used in the lamp. It follows clearly from these and other experiments that in the said cases the action cannot be ascribed to any active vapor, but only to the action of the introduced substance in a solid state. The present invention is based upon this conclusion.

The action of the solid substances upon the atomized particles from the incandescent wire striking their surface is probably due primarily to the formation of a solid 60 (colloidal) solution in the solid layer. Applicants however do not wish to bind themselves to this explanation. A favorable action of such substances is best realized when they are applied to the incandescent lamp 65 in such a place that they are struck by the particles ejected from the wire. Preferably therefore the surface of the substance in the bulb should be large. When however the stable substance is placed in a glass tube 70 or the like, as has been proposed for halogenids which dissociate by heat, it cannot act because the particles ejected from the wire will not strike it.

It is known that even small quantities 75 of water have a detrimental effect in a tungsten filament lamp. Therefore it is advantageous to choose non-hygroscopic substances, because smaller precautions are then necessary. As all soluble substances must 80 be considered hygroscopic, it is preferable to use substances which are insoluble in water.

In practice it has proven difficult to employ halogen or oxygen delivering substances in incandescent lamps burning under a high voltage of about 200 volts or higher, because arcing readily takes place between the feed wires. In the process according to the invention however no active vapor 85 pressure is necessary, but on the contrary would have a deleterious effect, especially in high voltage lamps, because it furthers arcing. Therefore it is preferable to use only slightly volatile and highly stable substances.

So for example calcium fluorid  $CaF_2$ , which is only slightly volatile and which is known to have a large degree of stability even at the temperature of the electric arc, 100 is especially fit for high voltage lamps. It has also the already mentioned advantage of being practically insoluble in water, in consequence of which this substance has no tendency to retain water or to absorb water 105 from a moist atmosphere.

An embodiment of the invention is illustrated in the accompanying drawing where-in a conventional type of electric lamp with the bulb in section, is shown. *a* designates 110 the filament supported in suitable manner within the glass bulb *b*. On the inner walls

of bulb *b* is a coating *c* of the substance, as calcium fluorid, which is used to counteract the blackening of the bulb. The thickness of the material *c* is shown much exaggerated 5 in the drawing, this layer being in fact of little thickness and invisible.

It has been proposed (U. S. Patent No. 406,130) to coat the inner surface of carbon filament lamps with a thin film of a substance mixed with more or less water, the substance being so chosen that the film becomes a good conductor of electricity, whereby the whole inner surface of the bulb is brought to the same potential as the filament 10 in order to prevent the electrical carriage 15 of material. The present invention, however, refers to an action obtained with a non-conducting film; all incandescent lamps in which a conducting film is applied upon 20 the surface of the globe, are expressly disclaimed.

It has been proposed (U. S. Patent No. 1,252,372) to coat the inner surface of the lamp bulb with a material, containing an 25 oxidizing agent, which at the temperatures encountered under operating conditions, is able to combine with the dark deposit, the resulting material being transparent. In this case the temperature of the active material 30 is much higher than the temperature of the bulbs of ordinary lamps of the vacuum type, because the active material is put on a surface, working as an "economizer", that is reducing the heat losses by 35 the hot gases in a gas-filled lamp. The present invention, however, refers to an action, obtained with a non-oxidizing sub-

stance, which does not reach a temperature higher than the bulb of an ordinary lamp of the vacuum type, all incandescent lamps 40 in which an oxidizing agent is applied upon the surface of the globe, being expressly disclaimed.

What we claim is:

1. An incandescent electric lamp of the 45 vacuum type comprising a bulb and a thin non-conducting layer on the inner surface of the bulb of a non-oxidizing substance which during the burning of the lamp does not evolve an active or measurable vapor 50 pressure of any gas, but prevents the obscuring of the bulb while solid.

2. An incandescent electric lamp of the 55 vacuum type comprising a bulb and a thin non-conducting layer on the inner surface of the bulb of a non-oxidizing substance which is practically insoluble in water and which during the burning of the lamp does not evolve an active or measurable vapor 60 pressure of any gas but prevents the obscuring of the bulb while solid.

3. An incandescent electric lamp of the 65 vacuum type comprising a bulb and provided on the inner surface of the bulb with a thin layer of fluorid of calcium.

In testimony whereof we have signed our names to this specification in the presence of two subscribing witnesses.

LODEWIJK HAMBURGER.  
DIRK LELY, JUNIOR.

Witnesses:

J. J. HELSDON RIX,  
ANN NAGTTANZEE.